

## UNITED STATES PATENT OFFICE

1,947,948

## METHOD FOR THE PRODUCTION OF ZINC SHEETS PARTICULARLY ADAPTED FOR USE IN GALVANIC CELLS

Paul Mittmann, Ludenscheid in Westfalen, Germany, assignor to American Lurgi Corporation, New York, N. Y., a corporation of New York

No Drawing. Application April 15, 1931. Serial No. 530,443, and in Germany April 19, 1930

6 Claims. (Cl. 148—11.5)

This invention relates to rolled sheet zinc, especially for cell cases and like electrotechnical purposes and to a method of manufacturing same.

Sheet zinc, such as is used for galvanic cells, for example, in the known cup or sleeve form, for anode batteries, must possess certain powers of resistance to the action of electrolytes, such as sulphuric acid. Such resistance is necessary, in order to assure sufficient durability of the finished, but unused cells, in storage, and for the uniform maintenance of the electromotive force. The testing of sheet zinc by the Cohen method has been elaborated on the basis of these considerations. Said test consists in immersing a plate of a given superficial area (25 sq. cm.) in a prescribed volume (100 cc.) of 10% sulphuric acid, and measuring the rise of temperature in the acid, which should exceed the initial temperature by 11–13° C. If the temperature has not risen above 3° C. in 30 minutes, the zinc is considered satisfactory. In reality, the Cohen test fully represents the requirements expected in practice with regard to the suitability of the sheet zinc for galvanic cells.

It has transpired in practice that no possibility existed up to the present, of producing sheet zinc in a form which always proved reliable under the Cohen test. On the contrary, it was found that though some of the sheets, from a parcel fairly satisfied requirements, the major portion of them always gave unsatisfactory results, and therefore could not be used at all, or at any rate, not for high-class articles. This behaviour of sheet zinc was hitherto ascribed to divergences in the properties of the material, it being considered that the origin of the brands of zinc used, the impurities, such as iron, lead, arsenic and the like, affected the suitability of the metal for the purposes in question. It has also been considered that the superficial structure of the plate, the compactness and the smoothness of the surface might be influential factors, though no one was able to say what the character of the plate ought to be, from this point of view, and what would be the effect of the various properties.

A specialist in these matters alleged that the Cohen test is the most sensitive for cell plates, and that plates which stood that test are suitable, in all circumstances, for articles of the highest quality. It is, however, not impossible that plates which do not fulfill the conditions of the Cohen test will occasionally give good results, but when such plates are used, the quality of the articles is entirely a matter of chance.

It has now been ascertained that rolled sheet zinc will always not only correspond to the Cohen conditions but will also far exceed the quality hitherto attained, according to the Cohen test, if the basal surfaces of the (hexagonal) zinc crystals in the plate lie parallel with the surface of the latter. Plates exhibiting this structure can be produced in different ways. For example, the microstructure prescribed according to the invention, can be obtained from sheets which have been rolled from the ordinary cast zinc slabs, if they are annealed at temperatures above 100° C., for example between 200° and 400°, followed by pressure treatment, preferably by cold rolling to the desired gauge. Zinc plates treated in this manner can always be relied on to pass the Cohen test.

Still better results are obtained when the casting of the zinc slabs is conducted in such a manner that the zinc crystals are disposed quite irregularly in the slabs. In contrast to the general casting process, this irregular disposition of the zinc crystals in the cast slab, is obtained by pouring the molten zinc at a temperature slightly exceeding the melting point, for example between 420° and 440° and preferably 430° C. This pouring temperature can be attained in a great variety of ways, for example by cooling molten zinc, that has been heated to a higher temperature, until it begins to solidify, or the production of this pouring temperature may be effected directly in heating the zinc placed in the melting furnace. For example, the furnace containing the charge of zinc may first be heated up until the zinc begins to melt, the fire being then drawn and the furnace left to itself for a short time, until the heat accumulated in the masonry and the like has assisted the fusion of the zinc to such an extent that 10–20% of the zinc charge can be scooped out of the furnace. The molten zinc is cast into slabs, preferably 10–11 mm. thick and weighing, when of the usual length and breadth, for example 17–18 kg. The fire is then ignited again, and working of the furnace and the pouring are resumed after suitable replenishment of the zinc.

This method of casting furnishes slabs consisting of very fine and irregularly disposed crystals, whereas in the usual casting process, all the zinc crystals are oriented to a certain extent. Since the basal surface of the hexagonal zinc crystal is a cleavage plane, the irregularly disposed small zinc crystals in these slabs arrange themselves, in the course of rolling, so that the basal surfaces lie on or parallel with the surface of the plates.

Under the Cohen test, plates produced in this manner give a rise in temperature of 1-2° C. in 30 minutes, and do not reach 30° C. until after 80-110 minutes. Thus, the zinc plates produced in 5 accordance with the invention give substantially better values, in the Cohen test, than the plates hitherto employed for galvanic purposes which, although they may pass the test to some extent, do not have the structure of the plates of the 10 invention. Moreover—and this constitutes the greatest technical advantage of the plates according to the invention, all the plates which exhibit the structure according to the invention, invariably fulfil the conditions of the test, whereas in 15 the case of the previous zinc plates, although, in some instances convertible into cell casings of high quality, there was no certainty that plates possessing these good properties could be produced, and no guarantee could be given as to 20 their quality. The orientation of the zinc crystals in the plate can be examined in accordance with known physical methods.

If it be desired to improve still further the plates produced from the slabs according to the 25 invention, this can be done by annealing the plates at the temperature already specified, followed by cold working.

The zinc plates according to the invention are 30 suitable, not only for galvanic purposes, but can also be employed with advantage in all cases where importance is attached to increased resistance of the zinc plates to corrosion.

I claim:—

1. A method for the production of zinc sheets 35 particularly adapted for use in galvanic cells which comprises casting relatively thin zinc plates at a temperature of from about 420°-440° C., roll-

ing said plates into sheets in the usual manner, and thereafter cold rolling the sheets.

2. A method for the production of zinc sheets 80 particularly adapted for use in galvanic cells which comprises casting relatively thin zinc plates from the molten portion of a charge of zinc at a temperature of from about 420° to 430° C. containing a substantial proportion of unmolten zinc, and rolling said plates into sheets in the usual manner.

3. A method for the production of zinc sheets 85 particularly adapted for use in galvanic cells which comprises casting relatively thin zinc plates from the molten portion of a charge of zinc at a temperature of from about 420° to 430° C. containing a substantial proportion of unmolten zinc, rolling said plates into sheets in the usual manner and thereafter cold rolling the sheets.

4. A method for the production of zinc sheets 90 particularly adapted for use in galvanic cells which comprises casting zinc plates at a temperature of from about 420 to 430° C. and rolling said plates into sheets in the usual manner.

5. A method for the production of zinc sheets 95 particularly adapted for use in galvanic cells which comprises casting zinc plates of not more than about 15 mm. thickness at a temperature of from about 420 to 430° C. and rolling said plates into sheets in the usual manner.

6. A method for the production of zinc sheets 100 particularly adapted for use in galvanic cells which comprises partially melting zinc, casting the molten zinc into plates at a temperature of about 430° C. and rolling the plates into sheets in the usual manner.

PAUL MITTMANN.

40

115

45

120

50

125

55

130

60

135

65

140

70

145

75

150